

## UNITED STATES PATENT OFFICE.

ALBERT L. KLEES, OF NEW YORK, N. Y., ASSIGNOR TO COMBUSTION UTILITIES CORPORATION, OF NEW YORK, N. Y., A CORPORATION OF MAINE.

## LUBRICATING COMPOSITION.

No Drawing.

Application filed July 18, 1924. Serial No. 726,278.

This invention relates to lubricating oils and particularly to a new and useful composition which possesses properties making it of exceptional value as a lubricant.

5 In true oil film or "viscous" lubrication, there is no slip between the solid and liquid surfaces and movement takes place by the intermediate planes of the liquid sliding over one another. The resistance to this shear 10 of plane over plane is due to the viscosity of the liquid. Efficient lubrication under all conditions has been found to depend upon the possession by the liquid of some other property which enables it further to reduce 15 the frictional resistance, and that property has been given the name of "oiliness." Mineral oils are as efficient lubricants under many conditions as animal or vegetable oils of similar viscosity and as they are more 20 inert chemically and are cheaper they are most widely used. There are, however, many conditions of operation and many parts of machinery in which a perfect oil film cannot form and in which the friction to be over- 25 come is due in large part to contact between solid and solid. Such a condition of incomplete lubrication occurs most frequently in bearings when starting from rest and when the load is exceptionally heavy. This static 30 friction in a bearing bears little or no relation to the viscosity of the lubricant, even when oils of the same class are used, and the character of the surfaces in contact has a great influence upon its magnitude. Mineral 35 oils and fatty oils show a great difference in behavior under these conditions. At the same pressure and temperature it has been found for example that under starting loads castor oil, which has a viscosity several times that of a heavier engine oil, nevertheless lowers the frictional resistance to a greater degree. This reduction of friction by lubricants such as castor oil has been ascribed to "oiliness", which property is possessed in greater degree by animal and vegetable oils than by ordinary mineral oils. Since different bearing metals have a widely different effect upon static frictional resistances, the theory has been advanced that "oiliness" is an effect produced by the lubricant upon the metallic surfaces with which it is in contact, rather than a property of the lubricant as a liquid. It has been found that the best lubricating mineral oils contain unsaturated molecules and it is well known that vegetable oils are usually glycerol esters of unsaturated fatty acids. It is believed therefore that the unsaturated molecules of the lubricant may enter into a firm physico-chemical union with the exposed metal, forming a bearing surface which is composed of both oil and metal.

The primary object of the present invention is to provide a lubricating composition which is superior both in the property of "oiliness" and as a dispersing medium for finely divided particles of material of unctuous properties.

Another object of the invention is to provide a lubricating composition the properties of which can be readily varied to meet varying conditions of "viscous" or oil film lubrication.

Another object of the invention is to provide a lubricating composition which can be advantageously used in admixture with petroleum products to improve their properties of "oiliness."

With these and other objects in view the present invention consists in the new lubricating composition hereinafter described and particularly defined in the claims.

The composition forming the subject matter of the present invention may be described briefly as consisting of a mixture of neutral oils, insoluble in alkali and dilute mineral acids and having a particular chemical constitution, either with or without ordinary petroleum lubricating oils and/or hydrocarbon oils of high temperature tar origin and/or high boiling tar-acids and/or graphite or other unctuous material. The neutral oils are characterized by the presence in large proportions of cyclic unsaturated non-benzenoid or hydro-aromatic hydrocarbons, which are related to the benzene-naphthalene series of compounds such as are found in ordinary coke-oven tar but which have a larger content of hydrogen and usually of alkyl groups and hence have a higher molecular weight, a lower density, and a lower refractive index for the same boiling point. These neutral tar oils differ further from the above-named aromatic (benzene-naphthalene) hydrocarbons by their ability to decolorize dilute solutions of potassium permanganate or bromine. They differ also from petroleum products in both their chemical and physical properties, since they are essentially primary distillates of coal or

other bituminous material and are formed only when the coal is distilled under low temperature conditions of carbonization. The tar-acid group which is sometimes used 5 in making up the above composition is composed of cyclic organic hydroxy compounds, soluble in alkali, of which at least 50% boil above 220° C. These compounds resemble the higher phenolic homologues which occur 10 in very small quantities in ordinary coke-oven tar, but differ from them by virtue of a larger content of hydrogen and of alkyl groups which give them a higher molecular weight, a lower density and a lower refractive index for the same boiling point.

The component groups which make up the present composition each have distinct functions to perform and their relative proportion in the final mixtures may be varied at 15 will to suit the requirements of various lubricating conditions. The neutral tar oils which contain cyclic unsaturated non-benzenoid hydrocarbons have been found to possess in high degree the property of uniting 20 with bearing surfaces to form an intermediate oily film of extremely low frictional resistance, and this property of "oiliness" is of particular advantage in that it reduces starting friction and permits the employment 25 of bearing loads far in excess of those which can be used with ordinary viscous lubrication. The mineral oils of petroleum origin often possess a high viscosity but rarely have the property of oiliness to any 30 marked extent. For this reason lubricants comprising a blend of the unsaturated neutral tar oils with petroleum oils are particularly valuable in that they may be compounded so as to possess "viscous" and 35 "oily" properties to meet almost any condition of ordinary lubrication. The cyclic organic hydroxy compounds or primary tar acids have been found to increase the viscosity of the neutral tar oils, and accordingly 40 are used in compositions where it is desired to establish conditions more nearly approaching viscous lubrication. For conditions involving unusually high pressures where it is necessary to disperse in the oils solids of 45 unctuous properties, it has been found that the neutral tar oils described above are of 50 particular merit because of their natural adaptability as dispersing mediums and further because they possess in favorable combination the properties of oiliness, low volatility and low viscosity. A low viscosity is 55 particularly advantageous in this connection because of the decreased resistance to internal shear within the liquid itself.

60 This group of neutral tar oils, a mixture of which in proper proportions with the other materials named comprises the present invention, can be prepared from the essentially primary or only partially decomposed primary tar obtained by distillation

of coal, oil shale or other bituminous material under conditions such as to prevent extensive secondary reactions, for example conditions such as are described in United States Patent No. 1,426,159 granted August 15, 1922, to Henry L. Doherty or in the British patent of Henry O. Loebell #216,488 of May 23, 1923, but which conditions are quite different from those which give rise to ordinary coke-oven tar. The tar obtained in either of the above processes is essentially a primary liquid distillate of the fuel, and as a result of the fractional distillation of the bituminous material solely by heat carried by a hot gas current, this tar contains the volatile components of the coal or other material in a primary or at most an only partially decomposed condition. This tar oil is therefore clearly distinguishable in both its physical and chemical properties from coke-oven tar and possesses an altogether different chemical composition.

The primary or partially decomposed primary tar obtained in the above processes is dehydrated and then distilled, either to pitch or coke, and the distillates thus obtained are treated to produce the neutral oil lubricants in question. Briefly this treatment comprises washing with a caustic alkali in either equivalent or insufficient proportions, depending on whether it is desired to remove all or only a portion of the cyclic hydroxy compounds present in the distillate. The neutral tar oil remaining after this treatment can be further treated to remove wax or otherwise to improve its properties by the application of methods similar to those generally employed in refining lubricating stocks from petroleum oil.

The proportion of unsaturated hydrocarbons in these essentially primary tar oils varies from about fifty percent in oils taken from the most primary type to over eighty percent in oils from tars that have been partially decomposed. Apparently it is the high content of cyclic unsaturated non-benzenoid hydrocarbons in these neutral tar oils which is mainly responsible for the greatly increased property of "oiliness" which they exhibit either when used alone or when compounded with petroleum lubricants.

In preparing a mixture of these neutral tar oils with ordinary petroleum oil for the purpose of securing a product containing the proper ratio of "oily" and "viscous" properties to meet the requirements of any particular condition, the viscosity of the compounded oil may be reduced below that found necessary to maintain a continuous layer between the rubbing surfaces under the existing conditions of rotational speed and bearing pressure. For light loads the neutral tar oils which are obtained by removing tar-acids and wax from the high-boiling distillates have sufficient viscosity in themselves to make

them entirely satisfactory. As a cheaper lubricant for unexacting conditions the fractions containing the higher boiling non-corrosive members of the tar-acid group which are present in the original distillate can be used in natural blends, or these high boiling primary tar acids can be esterified (as by benzene-sulfonic acid) to produce more viscous products. The middle-boiling neutral 10 tar-oils are peculiarly adapted for use as a vehicle for graphite or other dispersed solid lubricant, not only because of their particular adaptability as dispersing media but also because in their natural form they possess a 15 very favorable combination of the properties of low volatility and low viscosity.

The following examples are cited as being representative of some of the types of lubricants which may be made:

20 (a) For ordinary viscous lubrication:

10-40% of primary tar acids of which at least 50% boil above 220° C.; 30-60% of cyclic unsaturated non-benzenoid hydrocarbons; the balance consisting of dead or chemically inactive oils of similar boiling range containing naphthenic, paraffinoid or other saturated hydrocarbons together with small quantities of impurities such as nitrogen and sulphur-containing compounds.

30 (b) For oily or greasy lubrication:

Less than 10% high-boiling primary tar acids; 45-85% of high-boiling cyclic unsaturated non-benzenoid hydrocarbons; the balance consisting of naphthenic and paraffinoid hydrocarbons of similar boiling range containing small amounts of impurities; and the whole in blend with varying proportions of ordinary petroleum lubricants.

40 (c) For oily or greasy lubrication under extreme conditions a composition such as described in (b) above used as a dispersing medium for finely divided or colloidal graphite or other unctuous material, 0.25% (twenty-five hundredths per cent) of which is a favorable proportion.

It is not intended that the invention should be so limited in scope as to include only compositions containing the neutral tar-oils and high-boiling tar-acids which are obtained from a primary liquid distillate of bituminous material such as is produced by the Doherty or Loebell processes above referred to, since any oil can be used which contains cyclic unsaturated non-benzenoid hydrocarbons of similar nature, no matter by what means it is produced, so long as it contains said hydrocarbons in amounts sufficient to impart the requisite property of "oiliness" to the final lubricating composition.

60 The cyclic unsaturated non-benzenoid hydrocarbons which make up a large proportion of the neutral tar oils used in compounding the above lubricants, are not claimed as such in the present application. These cyclic unsaturated hydrocarbons are believed to be

essentially new compositions of matter which have not been heretofore known to the art, but as they possess properties which make them particularly valuable in compounding flotation oils, they have been specifically 70 claimed in my co-pending application for "flotation oils," filed June 7, 1924, Serial No. 718,674.

The term primary tar acids as used in the claims is intended as a generic term to describe the mixture of high-boiling tar-acids which are to be found in an essentially primary tar such as that described. Accordingly, this term primary tar acids is used generically to describe the high boiling alkali soluble hydroxy compounds 80 closely related to the phenols and comprising hydrogenated and alkylated or both hydrogenated and alkylated derivatives of phenol and phenol homologues which are 85 present in such tar oils, and of which at least 50% boil above 220° C.

The term "cyclic unsaturated non-benzenoid hydrocarbons" as used in the claims is intended as a generic term to describe 90 the mixture of cyclic unsaturated non-benzenoid hydrocarbons which make up a large proportion of the neutral oil fraction of such primary tar oils, and which are hydrogenated or alkylated or both hydrogenated 95 and alkylated derivatives of benzene, naphthalene, anthracene and homologous cyclic and polycyclic hydrocarbons of the benzene-naphthalene series.

The term "dead oils" as used in the specification is intended to describe the small proportion of hydrocarbons in the neutral oil fraction of primary tars which are not cyclic unsaturated hydrocarbons, but which consist principally of saturated paraffins 100 and naphthenes.

The preferred form of the invention having been thus described, what is claimed as new is:

1. A lubricating composition containing 110 cyclic unsaturated non-benzenoid hydrocarbons in admixture with naphthenic and paraffinoid hydrocarbons of similar boiling range.

2. A lubricating composition containing 115 cyclic unsaturated hydrocarbons, naphthenic and paraffinoid non-benzenoid hydrocarbons of similar boiling range, and primary tar acids of which at least fifty percent distil above 220° C.

3. A lubricating composition containing 120 cyclic unsaturated non-benzenoid hydrocarbons in admixture with a petroleum oil lubricant.

4. A lubricating composition containing 125 cyclic unsaturated non-benzenoid hydrocarbons and naphthenic and paraffinoid hydrocarbons in admixture with a petroleum oil lubricant.

5. A lubricating composition containing 130

- cyclic unsaturated non-benzenoid hydrocarbons, high boiling primary tar acids and a petroleum oil lubricant.
6. A lubricating composition containing 5 cyclic unsaturated non-benzenoid hydrocarbons and a small amount of graphite.
7. A lubricating composition containing 10 cyclic unsaturated non-benzenoid hydrocarbons, high-boiling primary tar acids, and graphite.
8. A lubricating composition containing 15 cyclic unsaturated non-benzenoid hydrocarbons, a petroleum oil lubricant, and graphite.
9. A lubricating composition containing 20 cyclic unsaturated non-benzenoid hydrocarbons, primary tar acids, a petroleum oil lubricant and a small amount of graphite.
10. A lubricating composition containing 25 more than ten percent high-boiling primary tar acids and more than thirty percent cyclic unsaturated non-benzenoid hydrocarbons.
11. A lubricating composition containing 30 more than ten percent primary tar acids and more than thirty percent cyclic unsaturated non-benzenoid hydrocarbons together with a lubricating oil of petroleum origin.
12. A lubricating composition containing primary tar acids of which at least fifty
- percent boil above 220° C., and more than forty-five percent of cyclic unsaturated non-benzenoid hydrocarbons.
13. A lubricating composition containing 35 primary tar acids, and more than forty-five percent of cyclic unsaturated non-benzenoid hydrocarbons in a blend with a petroleum oil lubricant.
14. A lubricating composition containing 40 more than forty-five percent of cyclic unsaturated non-benzenoid hydrocarbon tar oils in a blend with a petroleum oil lubricant.
15. A lubricating composition containing 45 at least forty-five percent cyclic unsaturated non-benzenoid hydrocarbons together with about twenty-five one-hundredths percent of finely dispersed or colloidal graphite.
16. A lubricating composition containing 50 at least forty-five percent of cyclic unsaturated non-benzenoid hydrocarbons in admixture with a petroleum oil lubricant and a small amount of finely dispersed graphite.
17. A lubricating composition containing 55 cyclic unsaturated non-benzenoid hydrocarbons and hydrocarbon oils of high temperature coal tar origin.

In testimony whereof I affix my signature.

ALBERT L. KLEES.

**CERTIFICATE OF CORRECTION.**

Patent No. 1,727,109.

Granted September 3, 1929, to

ALBERT L. KLEES.

It is hereby certified that error appears in the printed specification of the above numbered patent requiring correction as follows: Page 3, line 83, for the word "and" read "or"; same page, line 116, claim 2, after the word "unsaturated" insert the compound word "non-benzenoid", and line 117, strike out "non-benzenoid"; and that the said Letters Patent should be read with these corrections therein that the same may conform to the record of the case in the Patent Office.

Signed and sealed this 29th day of October, A. D. 1929.

M. J. Moore,  
Acting Commissioner of Patents.

(Seal)

- cyclic unsaturated non-benzenoid hydrocarbons, high boiling primary tar acids and a petroleum oil lubricant.
6. A lubricating composition containing 5 cyclic unsaturated non-benzenoid hydrocarbons and a small amount of graphite.
7. A lubricating composition containing 10 cyclic unsaturated non-benzenoid hydrocarbons, high-boiling primary tar acids, and graphite.
8. A lubricating composition containing 15 cyclic unsaturated non-benzenoid hydrocarbons, a petroleum oil lubricant, and graphite.
9. A lubricating composition containing 20 cyclic unsaturated non-benzenoid hydrocarbons, primary tar acids, a petroleum oil lubricant and a small amount of graphite.
10. A lubricating composition containing 25 more than ten percent high-boiling primary tar acids and more than thirty percent cyclic unsaturated non-benzenoid hydrocarbons.
11. A lubricating composition containing 30 more than ten percent primary tar acids and more than thirty percent cyclic unsaturated non-benzenoid hydrocarbons together with a lubricating oil of petroleum origin.
12. A lubricating composition containing primary tar acids of which at least fifty
- percent boil above 220° C., and more than forty-five percent of cyclic unsaturated non-benzenoid hydrocarbons.
13. A lubricating composition containing 35 primary tar acids, and more than forty-five percent of cyclic unsaturated non-benzenoid hydrocarbons in a blend with a petroleum oil lubricant.
14. A lubricating composition containing 40 more than forty-five percent of cyclic unsaturated non-benzenoid hydrocarbon tar oils in a blend with a petroleum oil lubricant.
15. A lubricating composition containing 45 at least forty-five percent cyclic unsaturated non-benzenoid hydrocarbons together with about twenty-five one-hundredths percent of finely dispersed or colloidal graphite.
16. A lubricating composition containing 50 at least forty-five percent of cyclic unsaturated non-benzenoid hydrocarbons in admixture with a petroleum oil lubricant and a small amount of finely dispersed graphite.
17. A lubricating composition containing 55 cyclic unsaturated non-benzenoid hydrocarbons and hydrocarbon oils of high temperature coal tar origin.

In testimony whereof I affix my signature.

ALBERT L. KLEES.

**CERTIFICATE OF CORRECTION.**

Patent No. 1,727,109.

Granted September 3, 1929, to

ALBERT L. KLEES.

It is hereby certified that error appears in the printed specification of the above numbered patent requiring correction as follows: Page 3, line 83, for the word "and" read "or"; same page, line 116, claim 2, after the word "unsaturated" insert the compound word "non-benzenoid", and line 117, strike out "non-benzenoid"; and that the said Letters Patent should be read with these corrections therein that the same may conform to the record of the case in the Patent Office.

Signed and sealed this 29th day of October, A. D. 1929.

M. J. Moore,  
Acting Commissioner of Patents.

(Seal)